

## UNITED STATES PATENT OFFICE

THEODOR HELLTHALER, OF GRANSCHUTZ, GERMANY, ASSIGNOR TO THE FIRM A. RIEBECK'SCHE MONTANWERKE AKTIENGESELLSCHAFT, OF HALLE, SAALE, GERMANY

## PROCESS FOR BLEACHING MONTAN WAX

No Drawing. Application filed July 18, 1927, Serial No. 206,799, and in Germany July 26, 1926.

This invention relates to the process of bleaching so-called montan wax. This mineral in chemical and physical respect resembles vegetable waxes, for instance carnauba wax. However the dark color of the montan wax is a great draw-back in comparison with vegetable waxes. Many attempts have been made to effect the bleaching of montan wax by physical and chemical treatment. Up to-date the wax is distilled in vacuo with superheated steam whereby a clear product is obtained; however, the output is quite unsatisfactory, and besides the chemical composition of the distillate differs from that of the raw material to a considerable extent. Therefore further trials were made to refine the montan wax solely by chemical means, but the outputs of such methods were likewise very small owing to the extensive formation of resins.

It has recently been proposed to bleach montan wax by chromic acid in presence of glacial acetic acid. With this oxidant it is possible to obtain a satisfactory output of a clear product which substantially conserves the character of the original wax. However, the relatively high price of glacial acetic acid as well as its unpleasant properties prevent a general application of this process which is therefore not carried out on an industrial scale.

Now I have found that montan wax can also be bleached by treating it with oxidants such as hydrogen peroxide, chromic acid or an alkali metal bichromate in presence of diluted sulfuric acid. When stirring montan wax in the molten state with oxidants in presence of diluted acid, the wax is strongly swelled up and emulsified in the diluted acid. In the state of distribution the montan wax offers the oxidants a surface of attack which otherwise only exists in the state of real solution. Suitable concentrations and conditions of working are described in the examples given at the end of the specification. However, my invention is not confined to these conditions which may be varied within wide limits without departing from the scope of my invention.

After the darkening constituents of the

montan wax have been oxidized, the cleared montan wax and the sulfuric acid separate into two distinct layers from which the upper, consisting of wax may easily be removed.

As the resinous constituents of the raw montan wax are violently attacked by the oxidizing agent, whereby less valuable products are formed, it is advisable to separate the resins from the montan wax by any known process before the oxidative treatment, especially when a montan wax rich in resins is to be treated. The preliminary separation of the resins affords the further advantage of saving oxidizing agents. As a result the thickening phenomena which disturb the uniform action of the oxidizing liquor and which otherwise can be avoided only with difficulty are reduced to a minimum.

In order to obtain products having special properties, the single constituents of the montan wax obtained by fractionating the wax by means of organic solvents, for instance the particularly valuable and easily clearable wax esters, may be treated according to my present invention, instead of using the whole or refined montan wax. In the same manner the wax alcohols and acids obtained by saponifying montan wax or the products obtained by transforming these substances may be subjected to the bleaching process.

The degree of clearing produced by my present process depends of course upon the constitution of the raw material, the amount of the oxidant employed and the method of operating. The treatment may be based, for instance, upon the counter-current principle, i. e. the raw material, which is, of course, more easily attacked by the oxidant than a wax already partially oxidized, is at first treated with a partially exhausted oxidative mixture, whereupon the partially oxidized wax is subjected to the action of fresh oxidative mixture until the desired bleaching effect is attained. In this way the oxidant will be completely utilized and, at the same time, a high bleaching effect obtained.

55

60

65

70

75

80

85

90

95

100

Rational and uniform oxidation may further be favoured by the addition of inert inorganic or organic distributors. For this purpose solid substances such as silica or, 5 earths, as well as especially inert liquid wax solvents, for instance carbon tetrachloride, may be used. These solvents are also suitable for checking the thickening phenomena which readily occur during the oxidation. 10 Of course, the distributors must be removed from the bleached wax by allowing them to set or by filtering or distilling.

After being treated with diluted sulfuric acid the wax still retains a certain amount 15 of sulfuric acid or reduced oxidant. For instance, when employing chromic acid as oxidant, the cleared wax is colored green by a chromic sulfate solution. For further refinement the wax may be treated in the 20 molten state with diluted acids and finally with water. If required, the last remnants of coloring contaminations may be removed by treating the wax either molten or dissolved in a suitable solvent such as benzene, 25 benzine, carbon tetrachloride with small quantities of an absorbent, for instance, floridine, color-removing carbon or the like. The output of products cleared according to my new process amounts to 88-96%. The 30 products retain their valuable physical properties and are of a light-yellow to white color, which depends upon the amount of the oxidant employed. The high fusing point so important for the value is conserved or even 35 increased under the oxidative treatment provided the oxidation is not overdone.

The sulfuric solution of the consumed oxidant obtained by the present process may be reoxidized in the well-known manner and then re-used.

#### 40 Examples

1. 500 grams of raw black-colored montan wax are melted and mixed with a solution of 1250 grams of concentrated sulfuric acid in 680 grams of water. With continuous stirring a solution of 500 grams of sodium bichromate in 500 grams of water is added within 4 hours. Stirring is continued 50 until the solution has become dark green. After stopping the stirrer the oxidized wax rises to the top of the chromic liquor and is removed. After melting and washing with a 10% sulfuric acid and finally 55 with water a yellow wax is obtained, the output amounting to 90%.

2. The same operations as in the foregoing example, but using a montan wax freed from resins in the well-known manner. A 60 yellow wax is obtained.

3. Raw montan wax is saponified and the non-saponifiable part removed from the soaps by a volatile solvent. The non-saponifiable part forms a substance yellow as wax 65 and fusing at 77° C. It may be further

cleared up by oxidation as above described.

The dark brown wax acids obtained by decomposing the soaps with mineral acids are converted, according to the foregoing examples, to light-yellow products, 100% 70 of sodium bichromate being employed for this purpose. The products show a fusing point of 83° C. and a saponification number of 150. The output amounts to 91%.

I claim:—

1. Process for bleaching montan wax which comprises treating the wax with an oxidant in presence of moderately diluted sulfuric acid.

2. Process for bleaching montan wax which comprises extracting the resinous matter from the wax and then treating the wax with an oxidant in presence of moderately diluted sulfuric acid.

3. Process for bleaching montan wax which comprises isolating the constituents of the wax by means of solvents, and separately treating the said constituents with an oxidant in presence of moderately diluted sulfuric acid.

4. Process for bleaching montan wax which comprises treating the wax partially exhausted and then with a fresh oxidant in presence of moderately diluted sulfuric acid.

5. Process for bleaching montan wax which comprises treating the wax with an oxidant in presence of moderately diluted sulfuric acid and a distributing medium.

6. Process for bleaching montan wax which comprises treating the wax with an oxidant in presence of moderately diluted sulfuric acid and washing the product with a diluted acid and thereafter with water.

7. Process for bleaching montan wax which comprises treating the wax with an oxidant in presence of moderately diluted sulfuric acid, dissolving the product in the presence of a decolorizing solid absorbent, separating the solution from the said solid adsorbent, and removing the solvent employed.

8. Process for bleaching montan wax which comprises isolating the constituents of the wax by means of solvents, separately treating the said constituents with an oxidant in presence of moderately diluted sulfuric acid, dissolving the product in an inert organic solvent in the presence of a decolorizing solid absorbent, separating the solution from the said solid absorbent, and removing the solvent employed.

9. Process for bleaching montan wax which comprises treating the wax with an oxidant in presence of diluted sulfuric acid containing about 65%  $H_2SO_4$ .

10. Process for bleaching montan wax which comprises extracting the resinous matter from the wax and then treating the wax with an oxidant in presence of diluted sulfuric acid containing about 65%  $H_2SO_4$ .

11. Process for bleaching montan wax which comprises fractionating the constituents of the wax by means of solvents, and separately treating the said constituents with an oxidant in presence of diluted sulfuric acid containing about 65%  $H_2SO_4$ .
12. Process for bleaching montan wax which comprises treating the wax with a partially exhausted and then with a fresh oxidant in presence of diluted sulfuric acid containing about 65%  $H_2SO_4$ .
13. Process for bleaching montan wax which comprises treating the wax with an oxidant in presence of diluted sulfuric acid containing about 65%  $H_2SO_4$ , and a distributing medium.
14. Process for bleaching montan wax which comprises treating the wax with an oxidant in presence of diluted sulfuric acid containing about 65%  $H_2SO_4$  and washing the product with a diluted acid and thereafter with water.
15. Process for bleaching montan wax which comprises treating the wax with an oxidant in presence of diluted sulfuric acid containing 65%  $H_2SO_4$ , dissolving the product in an inert organic solvent in the presence of a decolorizing solid absorbent, separating the solution from the said solid absorbent, and removing the solvent employed.
16. Process for bleaching montan wax which comprises fractionating the constituents of the wax by means of solvents, separately treating the said constituents with an oxidant in presence of diluted sulfuric acid containing about 65%  $H_2SO_4$ , dissolving the product in an inert organic solvent in the presence of a decolorizing solid absorbent, and removing the solvent employed.
17. Process for bleaching montan wax which comprises treating the wax with an oxidant in presence of diluted sulfuric acid containing about 65%  $H_2SO_4$  dissolving the product in the presence of a decolorizing solid absorbent, separating the solution from the said solid absorbent, and removing the solvent employed.
18. Process for bleaching montan wax which comprises fractionating the constituents of the wax by means of solvents, separately treating the said constituents with an oxidant in presence of diluted sulfuric acid containing about 65%  $H_2SO_4$ , dissolving the product in an inert organic solvent in the presence of a decolorizing solid absorbent, separating the solution from the said solid absorbent, and removing the solvent employed.
- 60 In testimony whereof I affix my signature.

THEODOR HELLTHALER.